

Sept. 17, 1929.

J. H. DEPELER

1,728,232

WELDING RAJLS UNDER TRAFFIC

Filed Sept. 8, 1928

*Fig. 1*



*Fig. 2*



INVENTOR

*John H. Deppeler*  
BY  
*James S. Davis*

HIS ATTORNEY

## UNITED STATES PATENT OFFICE

JOHN H. DEPELER, OF WEEHAWKEN, NEW JERSEY

## WELDING RAILS UNDER TRAFFIC

Application filed September 8, 1928. Serial No. 304,795.

The invention relates to certain new and useful improvements in the alumino-thermic welding of rails under traffic, the invention comprising the fixing of the adjacent rail 5 ends against relative movement by forcing a locking member, preferably in the form of a wedge, vertically between the ends of the rail heads to effect notched engagement therewith and also to place the rails under 10 heavy compression, which will be effective, when the alumino-thermic metal is cast about the parts, to produce a pressure weld between the locking member and the rail ends.

The accompanying drawings illustrate 15 two modes of applying the locking member.

Fig. 1 is a side elevation of the rail ends and the locking wedge in the process of insertion between the rail heads.

Fig. 2 is a similar view showing a wedge 20 flanked by shims.

In the welding of rails by the alumino-thermic method without interrupting traffic, the most important problem met is to provide means for locking the rail ends together, 25 so that there can be no relative motion of the rail ends during the welding operation and during the preparatory work before the actual welding regardless of the number of wheel loads passing over the joint. In a 30 previous application, Serial No. 250,201, filed on the 28th day of January, 1928, there is disclosed a mode of fixing the adjacent rail ends against relative movement, which, in its specific application, involves the formation 35 of transverse notches in the rail webs and forcing a wedging member into bridging engagement with said notches. The present invention is designed to afford a somewhat simpler mode of locking the rail ends against 40 relative movement and at the same time imposing on the rails longitudinal compressive stresses which will be effective in producing a homogeneous pressure weld when the superheated molten metal is teemed about the 45 ends to form the joint.

Referring to Fig. 1, the numerals 1 and 2 indicate the ends of the rails to be welded together, the webs and bases of the rails being separated by a standard gap 3, while the 50 rail heads are separated by a smaller gap

4. Into the latter is driven, in a vertical direction, a locking member 5, preferably in the form of a wedge of steel. As the rails are fastened to the cross ties and because of the driving in of the wedge 5 until the top thereof is substantially flush with the rail treads, the effect will be to cause a notched engagement between the end faces of the rail heads and the wedge and will not only lock the rails against relative movement, but will also impose a heavy longitudinal compressive stress on the rails, so that, when the superheated alumino-thermic metal is cast about the rail ends, in the usual type of mold employed for this purpose, the rail ends and the interposed wedge or locking member are raised to welding temperature and because of the compressive force applied to the rails by the wedge, an effective pressure weld will be produced between the ends of the rail heads and the 55 locking member 5, the other elements of the rail ends being united by the alumino-thermic metal when the latter cools.

As illustrated in Fig. 2, the adjacent ends of the rails to be welded are separated 60 throughout by a standard gap 3 and the rails are locked together to prevent any relative movement by means of a steel wedge 5', which is flanked by shims 6, 6 of soft iron or mild steel, so that, when the wedge is 65 driven home, traffic may proceed uninterruptedly over the joint. In this case, the interlock is formed by the notching of the steel of the rail heads and of the wedge into the soft iron shims, and the latter serve to produce a more effective and homogeneous pressure weld between the steel of the rail heads and the steel of the wedge when the alumino-thermic metal is teemed about the joint as 70 before described.

What I claim is:

1. The method of welding rails which comprises fixing the adjacent rail ends against relative movement by forcing a locking member vertically between the ends of the rail heads to effect notched engagement therewith and exert a longitudinal compressive force on the rails, and casting alumino-thermic metal about the parts to produce a 75 80 85 90 95 100

pressure weld between the locking member and the rail ends.

2. The method of welding rails which comprises fixing the adjacent rail ends against relative movement by forcing a metal wedge vertically between the ends of the rail heads to effect notched engagement therewith and exert a longitudinal compressive force on the rails, and casting alumino-thermic metal about the parts to produce a pressure weld between the wedge and the rail ends.

3. The method of welding rails which comprises fixing the adjacent rail ends against relative movement by forcing a steel wedge flanked by iron shims vertically between the ends of the rail heads to effect notched engagement between the several elements and exert a longitudinal compressive force on the rails, and casting alumino-thermic metal about the parts to produce a pressure weld between the wedge and the rail ends.

In testimony whereof I affix my signature.

25 JOHN H. DEPPELER.